

## 1

3,304,223

ELIMINATING HYDROGEN SULFIDE ODOR  
DURING THE PROCESS OF FORMING WET  
STRENGTH PAPER CONTAINING CEREAL  
XANTHATESDonald H. Wheeler, Minneapolis, Minn., assignor to General Mills, Inc., a corporation of Delaware  
No Drawing. Filed Apr. 16, 1964, Ser. No. 360,415  
4 Claims. (Cl. 162—175)

The present invention relates to a process of paper manufacture which involves the use of cereal xanthates as wet strength additives.

Cereal xanthates have recently been suggested as wet strength additives for paper products. To accomplish this, the cereal xanthate is cross-linked by the use of an oxidizing agent to form the xanthide. However, in this operation frequently  $H_2S$  is given off which is objectionable in most paper processing plants.

It has now been discovered that by means of the present invention it is possible to cross-link the cereal xanthate to the xanthide without the production of any objectionable quantities of  $H_2S$ . In addition, surprisingly enough it is found that the wet strength of the paper is improved by the present process as compared to certain prior suggested processes.

The reactions involved in the formation of the xanthate and the cross-linking of the xanthate to the xanthide are illustrated in the following equations:



In the above equations R is the residue of the starch molecule found in typical cereal starting material. The starting materials may be cereal starches, but because of the cost element, the starting material is preferably a low grade flour or a millfeed commonly referred to in the trade as bran. Because of its preference from a cost standpoint, the detailed description will be with particular reference to bran. In the xanthation reaction the bran may be reacted with the sodium hydroxide or other alkali metal hydroxide and the carbon disulfide either in the form of a dilute solution or dispersion or in the form of a concentrate in which event the xanthate is obtained in the form of a stiff gel or as a particulate moist powder at low levels of water content. In either event a solution of the xanthate is used in the paper making operation. The xanthate solution is added to the pulp and dispersed therein. In certain prior art processes the pH of the pulp dispersion has been adjusted to 7 or even down to 4 or 5 by the addition of acid and then an oxidizing agent is added for the purpose of cross-linking the xanthate to the xanthide. A variety of oxidizing agents may be used for this purpose but chlorine or the hypochlorite are preferred for reasons of ready availability and economy. When this process is carried out it is found that rather large amounts of  $H_2S$  are evolved in the neutralization step of the paper making operation and these are objectionable.

It has now been discovered, however, that it is possible to neutralize only part of the alkali used in preparing

## 2

the xanthate and to add then the cross-linking oxidizing agent and thus eliminate the problem of  $H_2S$ . In the preferred operation the cross-linking is effected by bubbling chlorine gas through the pulp dispersion which served the purpose, not only of cross-linking by oxidation but also served to acidify the pulp to a pH of 6 or lower.

Attempts were made in the past to use the chlorine both as an acidifying agent and as the cross-linking oxidant. Under these circumstances it was found that 10  $H_2S$  was not evolved but actually the quality of the paper was impaired as compared with the use of a regular mineral acid as a preliminary neutralizing agent prior to the use of the cross-linking oxidant. It has been found that when from 10% to about 65% of the alkali used in 15 forming the xanthate is neutralized by a strong mineral acid such as sulfuric or hydrochloric prior to the addition of a cross-linking oxidant that there is virtually no  $H_2S$  formed when the pulp is ultimately acidified and converted into paper. When less than about 10% of the 20 alkali is neutralized prior to the addition of the oxidant the improvement in wet strength falls off as compared with preliminary neutralization within the range of 10% to 65%. Likewise, when one attempts to neutralize more than about 65% of the alkali prior to the addition of the 25 oxidant, it is found that increasing quantities of  $H_2S$  are evolved.

The following examples will serve to illustrate the invention.

## Example 1

30 5 grams of ground bran, at 5% moisture (0.0293 mole of anhydroglucose units), was stirred with 50 ml. of  $H_2O$ . To this was added 2.9 ml. of 30% NaOH solution by weight (1 mole NaOH per anhydroglucose units of bran) and thoroughly mixed by stirring. To this mixture was 35 added 0.74 g. of  $CS_2$  (0.3 mole per anhydroglucose unit of bran). The reaction was allowed to proceed for 15 minutes at room temperature. The reaction mixture remained as a stirrable, pourable liquid at all stages.

40 The above dispersion was immediately added to 24 g. of unbleached sulphite paper pulp which was dispersed in 3.2 liters of water. The mixture of cellulose paper pulp and xanthate was partially neutralized by addition of 4 ml. of 10%  $H_2SO_4$  (approximately 32% of the  $H_2SO_4$  needed to neutralize the NaOH used in making the xanthate). Chlorine gas was then bubbled into the mixture with stirring until the pH was lowered to 6 (required 0.82 g. of  $Cl_2$ ). No odor of  $H_2S$  was observed during this acidulation, as well as during the oxidation by chlorine. The mixture was stirred for 15 minutes, after which it was made into hand sheets (3 sheets test paper) size 12 inches by 12 inches and weighing about 8 grams each. The sheets were pressed on a screen between felts and then dried in a steam heated dryer.

45 Similar sheets were made without the additive (control). The control and sample sheets were equilibrated in a room at 70° F. at 50% relative humidity. The sheets were then weighed in order to calculate tensile strength at identical sheet weights. The 4.75 g. of bran (dry basis) represents a 20% addition of bran as xanthate to the cellulose pulp. The control sheets were tested for mullin burst strength in the dry state for a reference value. The control sheets when immersed in  $H_2O$  for 1/2 hour gave wet burst of 1 to 2% of the dry burst. The sheets containing bran made according to this example gave wet burst of 39% of the dry control.

A series of examples were run in which variations were made in the relative amount of sodium hydroxide and carbon disulfide used in the xanthation and in which varying amounts of the NaOH were neutralized. The results are given in the following table:

|        | NaOH used in Xanthation moles/anhydroglucose unit | CS <sub>2</sub> used in Xanthation moles/anhydroglucose unit | NaOH Neutralized with H <sub>2</sub> SO <sub>4</sub> , percent | Wet Burst Strength, <sup>1</sup> Percent |
|--------|---------------------------------------------------|--------------------------------------------------------------|----------------------------------------------------------------|------------------------------------------|
| 1..... | 1.0                                               | 0.3                                                          | 16                                                             | 35                                       |
| 2..... | 1.0                                               | 0.3                                                          | 32                                                             | 39                                       |
| 3..... | 1.0                                               | 0.3                                                          | 49                                                             | 33                                       |
| 4..... | 1.0                                               | 0.3                                                          | 65                                                             | 28                                       |
| 5..... | 1.0                                               | 0.2                                                          | 32                                                             | 40                                       |
| 6..... | 1.0                                               | 0.2                                                          | 49                                                             | 35                                       |
| 7..... | 0.8                                               | 0.2                                                          | 49                                                             | 33                                       |
| 8..... | 1.0                                               | 0.1                                                          | 31                                                             | 19                                       |
| 9..... | 1.0                                               | 0.1                                                          | 49                                                             | 30                                       |
| 10.... | 1.0                                               | 0.3                                                          | 0                                                              | 25                                       |
| 11.... | 1.0                                               | 0.2                                                          | 0                                                              | 13                                       |

<sup>1</sup> With 20% bran xanthate added to paper; wet burst as percent of dry burst of control without additive.

It will be evident from the above table that various ratios of NaOH and CS<sub>2</sub> to anhydroglucose units may be employed, and similarly that the degree to which the NaOH is neutralized may be varied. The table also demonstrates that when the NaOH is not neutralized, at least in part prior to the addition of the chlorine the wet burst strength of the paper is impaired. The amount of xanthate used in the paper can be varied over considerable limits. Generally however it is preferred to employ at least 5% of the xanthate based on the weight of the paper and it may go as high as 40% or more of the weight of the paper. The particular quantity to be employed depends upon the particular degree of wet strength and other properties desired in the paper and the cost of the paper relative to the properties.

Numerous other modifications of the invention may be made without departing from the spirit thereof as defined in the following claims.

The embodiments of the invention in which an exclusive property or privilege is claimed are defined as follows:

1. In a process of making paper from a pulp slurry which includes the incorporation in the pulp slurry of an alkali metal xanthate selected from the group consisting of xanthates of cereal starches, flour and bran and cross-linking said xanthate by means of an oxidizing agent selected from the group consisting of chlorine and hypochlorite prior to the formation of paper from said slurry which process normally results in the liberation of objectionable quantities of H<sub>2</sub>S, the step of substantially eliminating the liberation of objectionable quantities of H<sub>2</sub>S which comprises neutralizing the alkali used in forming the xanthate to an extent of from about 10 to 65% of said alkali by means of a strong mineral acid.

2. Process according to claim 1 in which approximately 50% of the alkali used in forming the xanthate is neutralized prior to the addition of the oxidizing agent.

3. Process according to claim 1 in which the oxidizing agent is chlorine.

4. Process according to claim 1 in which the xanthate is employed in a proportion from about 5 to 40% based on the weight of the paper.

#### References Cited by the Examiner

##### UNITED STATES PATENTS

3,160,552 12/1964 Russell et al. ----- 162—175

##### OTHER REFERENCES

Russell et al.: Tappi, vol. 45, No. 7, July 1962, pp. 557—566.

DONALL H. SYLVESTER, Primary Examiner.

S. LEON BASHORE, Examiner.